# EUROPEAN PATENT SPECIFICATION

(11) **EP 2 101 333 B1**
(45) Date of publication and mention of the grant of the patent: **30.04.2014**
(21) Application number: 07852046.7
(22) Date of filing: 07.11.2007
(51) Int. Cl.: G21F 9/16

(54) **METHOD FOR LIQUID RADIOACTIVE WASTE REPROCESSING**
VERFAHREN ZUR UMVERARBEITUNG VON FLÜSSIGEN RADIOAKTIVEN ABFALLSTOFFEN
PROCÉDÉ DE TRANSFORMATION DE DÉCHETS RADIOACTIFS LIQUIDES

(30) Priority: 06.12.2006 RU 2006143293
(43) Date of publication of application: 16.09.2009
(73) Proprietor: Obschestvo S Ogranichennoi Otvetstvennostyu "Nauka - Tekhnologii - Proizvodstvo", Moscow 119992 (RU)
(72) Inventor: AVRAMENKO, Valentin Alexandrovich, Vladivostok, 690068 (RU); DOBRZHANSKY, Vitaly Georgievich, Vladivostok, 690092 (RU); SERGIENKO, Valentin Ivanovich, Vladivostok, 690068 (RU); SHMATKO, Sergei Ivanovich, Moscow, 117463 (RU)
(74) Representative: HOFFMANN EITLE
(86) International application number: PCT/RU2007/000614
(87) International publication number: WO 2008/069694

(56) References cited:
- DE-A1- 3 833 676
- JP-A- 06 160 593
- RU-C1- 2 185 671
- RU-C1- 2 185 671
- RU-C2- 2 212 069
- US-A- 5 926 771
- US-A1- 2002 038 070

## Description

### Technical Field

The invention relates to protection of the environment, namely methods for liquid radioactive waste (LRW) reprocessing comprising immobilizing same into a crystal material, acceptable from the viewpoint of ecology and the invention can be used at facilities of atomic power industry and chemical-metallurgical production lines.

### Background Art

Liquid radioactive waste reprocessing is connected with the necessity to attain a safe long-term storage of radioactive waste (RAW), for which purpose hard radioactive waste (HRW) change into a state providing for a minimum leaching-out of radionuclides with natural waters. This task is solved by conventional methods such as bituminization, cementation and vitrification of RAW (patent RU N 2088986, 27.08.1997; patent RU N 2271586, 10,03.2006; patent RU N 2131152, 27.05.1999; Donald I.W., Metcalfe B.L., Taylor R.N.J. The immobilization of high level radioactive wastes using ceramics and glasses. Review. Journal of Materials Science, 32, 1997. p. 5856-5862), The least degree of leaching is provided with RAW vitrification and has a value of about 10⁻⁶ g/cm. day.

By now a marked interest is shown in oxide materials as matrices for the concentration and solidification of solutions of radionuclides salts and heavy metals usable in processes for treatment of liquid radioactive wastes. Such a form of burial of waste material is most promising as affording higher radioactive, chemical and thermal stability as against the methods as mentioned hereinabove.

Such forms of RAW immobilization are ceramic material widely known by the trade name Syncron whose matrix is normally a combination of hollandite (BaAl₂Ti₂O₆ or BaAl₂Ti₆O)₆), perovskite (CaTiO₃) and zirconolite (CaZrTi₂O₇).

A great number of works are dedicated to the synthesis and use of ceramics Synroc for immobilizing RAW (patent RU N 2153717, 27.07.2000, EP N 0007236, 23.01.1980; US N 4274976, 23.06.1981; Ringwood A.E., Kesson S.E., Reeve K.D., Levins D.M., Ramm E.J. Synroc. In: Radioactive Waste Forms for the Future. Eds. Lutze W. and Ewing R.C. Amsterdam: Elsevier Science Publishers B.V., 1988. P. 233-334; Donald I.W., Metcalfe B.L., Taylor R.N.J. The immobilization of high level radioactive wastes using ceramics and glasses. Review. Journal of Materials Science, 32, 1997, p. 5862-5865 et al.). Materials of this type allow to reduce the degree of RAW leaching from a ceramic matrix up to 10⁻⁹ g/cm² .day.

Said methods of RAW reprocessing in which radio active wastes are immobilized into a ceramic matrix have, alongside the aforesaid advantages, some defects, which are attributable to the high power capacity of high-temperature processes carried out at 1000°C or higher, a multitude operations and the necessity to employ special equipment.

Besides, it should be noted that the use of ceramics Synroc is effective in the case of small RAW volumes being immobilized, highly active wastes (HAW) for the most part.

Document US5926771 discloses the use of hydroxyapatite as an ion exchanger for radwaste, wherein under hydrothermal conditions at room temperature a monolith formation for waste disposal takes place (cf. col.1 line 60-col.11 line 30, claims 1-6 and examples 1-7).

Document US2002/038070 discloses the use of apatite as immobilizing medium for radwaste and the crystal formation on the surface of the apatite particles (cf. para [0212] - [0217]).

However these documents are silent about the specific hydrothermal conditions and specific solid particles other then apatite or hydroxyapatite used for the recrystallization of synthesizable compounds containing radionuclides on the surface of the layer. The documents disclose the immobilization of radioactive waste combining thereof with the matrix from an insoluble material.

In recent years much work has been done on the hydrothermal synthesis of ceramic materials and minerals suitable for immobilizing radionuclides in RAW reprocessing.

A rate of crystal growth through hydrothermal synthesis is increased many a time as against synthesis at normal temperatures, which hydrothermal synthesis presents new opportunities for selectively recovering radionuclides, However, the number of ceramic materials hydrothermally synthesized and capable of immobilizing the radionuclides is very limited. (Johnson CD., Skakle J.M. S., Johnson M.G. Feldmann J. Macphee D.E. Hydrothermal synthesis, crystal structure and acqueous stability of two cadmium arsenate phases, CdNH4(HAsO4)OH and Cd5H2(AsO4)4·4H2O.J. Mater.Chem. 2003, 13, 1429-1432).

Hydrothermal methods of reprocessing radioactive wastes go to show that the basic problems of LRW hydrothermal purification from radionuclides are as follows:
- selection of a type of ceramic matrix produced due to hydrothermal synthesis, which should be selective toward the corresponding radionuclides;
- ceramic matrix is formed in treatable LRW media (pH, composition of salt and other) while introducing suitable agents into solution at predetermined temperatures and pressure in a system;
- separation coefficient "ceramics-solution" should be great enough for a coefficient to be provided to purify the solution from the radionuclides.

Sorption reactant materials (SRM) are the new promising materials for the recovery of radionuclides.

The principle of operation of sorption-reactant materials resides in continuously forming an insoluble compound sorbing radionuclides in a porous matrix of inert material, with a continuous growth of crystals of the insoluble compound concurrently with sorption of the radionuclides. The result: there form crystal materials with a very small interface surface and sorbed radionuclides distributed over entire volume of the crystal material; such being the case, the leaching of radionuclides from sorption-reactant materials is by several orders lower than from selective ion - exchange sorbents having a large exchange capacity and, as so, a large interface surface.

Thus, patent RU No 2185671 20.07.2002 discloses the recovery of strontium radionuclides from solutions with a high content of hardness salts and liquid radioactive wastes of a complex chemical composition. SRMs are formed directly in the process of purification due to reaction of a starting sorption-reactant material comprising barium exchange cations, with a sulfate-ion purifying containing solution with the formation of insoluble barium sulfate crystallzable in the matrix of the sorption-reactant material.

This method is the closest prior art to the method sought for protection.

### Disclosure of Invention

An object of the present invention is to provide of a method of reprocessing liquid radioactive wastes containing long-lived radionuclides, preferably cobalt, manganese and strontium in hydrothermal conditions, which provides a high degree of purification of solutions from radionuclides, as required, a high separation coefficient (a ratio of purified LRW/HRW volumes), formation of a strong durable ceramic matrix with a minimum leaching-out of the radionuclides.

The problem is solved by a method of reprocessing liquid radioactive wastes containing long-lived radionuclides by synthesis of insoluble compounds immobilizing the long-lived radionuclides into a crystal lattice under hydrothermal conditions in a flow by passing LRWs being treated and reagents required for the synthesis through a layer of transition metal oxides at a rate providing for crystallizing of synthesizable radionuclide-containing compounds on the surface of the particles of the layer of oxides.

The transition metal oxides used are represented by iron oxide and/or manganese oxide and/or cobalt oxide and/or zirconium oxide.

The conditions for hydrothermal synthesis are a temperature comprised between 180 and 250°C and a pressure between 2.026 to 15.2 MPa (20 and 150 atm).

Essence of the method according to the present invention consists in the following.

While passing a solution of LRWs and reagents through a layer of insoluble oxides in hydrothermal conditions, a new crystal phase is grown on layer forming oxide particles, which represents the compounds immobilizing radionuclides.

One of the distinctions; of a method is the fact that in hydrothermal conditions, the synthesis of insoluble particles is carried out through crystallization of a new phase on the surface of oxides of a layer, not in the volume of the layer, as in the case of a known method (RU 2185671).

The term "crystallization" as it understood here means the change of a substance from the liquid state to the solid crystal state and the term "crystallization on the surface of particles" is heterogenic formation of a crystal phase on the surface of a solid.

By the term "phase" in the context of the present invention one should imply a generally accepted in the art, uniform in formulation and properties, part of a thermodynamic system separated from other phases by interfaces on which some of the properties of the system change stepwise.

By the term "immobilization" in the present invention one should imply inclusion of radionuclides in a crystal lattice of insoluble compounds crystallizable on the surface of particles of a layer.

During the realization of a process, a solution of LRW is passed through a layer of particles and on the surface of the layer in hydrothermal conditions, more exactly, at elevated temperature and pressure, new compounds are synthesized in form of crystals which

immobilize radionuclides. The speed of passing of LRW solutions through the layer of particles should be such that the formation of crystals on the surface of the layer of immobilizing radionuclide particles provide the desirable degree of purification from the radionuclides. In the case the speed of a flow is greater than a certain value determined experimentally in each and every particular case there occurs crystallization in the volume of a solution but not the surface of particles of the layer and more than that a portion of radionuclides containing crystals are lift out of the layer and no purification occurs whatsoever.

For purification to be carried out a solution being treated should contain ions forming under hydrothermal conditions the crystals of compounds immobilizing radionuclides. For the synthesis of a crystal phase reagents which would supply presence with ions required for the synthesis in the solution are added to the solution of LRW, said reagents being represented by oxidants such as hydrogen peroxide or potassium permanganate, oxidizing ions within the LRWs to an oxidation state of formation of insoluble compounds, and/or metal salts.

As a result of a research it has been established that crystal synthesis depends on the concrete conditions of a hydrothermal process. Thus, given the equal speed of a stream on initial solution which does not exceed the speed of crystallization in a range of temperatures of from 180 to 250°C and pressure of from 2.026-15.2MPa (20 to 150 atm), crystallization occurs on the surface of particles of a layer.

In case of a process being realized at a pressure of not less than 2.026 MPa (20 atm) and a temperature of below 180°C, crystallization partially occurs in a volume. A process carried out at a pressure of above 15.2 MPa (150 atm) and a temperature of above 250°C is not justified economically.

For details see for explanations of a process using diagrams in Figs. 1-3.

Fig. 1 shows the ASM-pictures of particles of a layer before hydrothermal synthesis (initial particle), Fig. 2 - in the process of synthesis, Fig. 3 - upon completion of hydrothermal synthesis.

### Carrying out the Invention

A method for any one of the alternative embodiments is realized as followings.

Reagents as required depending on the type of the LRWs being processed are added to the feeding LRW followed by feeding LRWs to the flow reactor for hydrothermal synthesis in which a layer of particles of insoluble compounds is placed.

Synthesis is carried out in a temperature range of 180 to 250°C, at a pressure of 2.026-15.2MPa (20 to 150 atm), which corresponds to the sufficient rate of crystal growth and the desirable degree of purification from radionuclides.

The compounds resulting from hydrothermal synthesis are deposited on insoluble particles forming the layer.

Upon completion of a process, when all particles are covered by the crystals of synthesized compounds containing radionuclides, these are directed for storage or further treatment. A radionuclide-free solution is a process radioactive-free waste material.
Fig. 1 shows a process of purification during the initial time t. The speed of a LRW solution's flow is sufficient for forming crystals on the surface of particles of a fixed layer.
Fig. 2 shows a process in a timed interval t'. A new crystal phase in the form of layered polycrystals has formed on the surface of particles forming the layer of insoluble particles. This corresponds to realization of the process for purification in the most favourable conditions.
Fig. 3 shows the process in final time t" when layered polycrystals with immobilized radionuclides have been formed on all the insoluble particles.

The layered structure of a synthesized compound which grows on an initial globular structure is seen on the pictures.

It has been found that the degree of purification from radionuclides during the synthesis of oxides was 10² to 10⁴. A ratio of the volumes of LRWs being processed to the volume of the reactor partially filled with initial particles was 500-2000 or more, which fact corresponds to separation coefficients of more than 10⁶.

The invention is illustrated by the following examples.

EXAMPLE 1 (not forming part of the claimed invention; Variant 1). LRWs containing 2 g/l Trilon B and 0.5 g/l trisodium phosphate having a 0.1 g/l concentration of calcium ions and comprising strontium-90 radionuclides (1.5·10⁻⁶ Ci/l) are passed through a layer of hydroxylapatite Ca₃PO₄·Ca(OH)₂ having a particle size of 0.1-0.3 mm, charged into a heated cylindrical reactor dimensioned 100 x 10 mm. The process is carried out at the flow speed of I ml/min., at the temperature of 200°C and pressure of 100 atm (10.13 MPa). A solution flow is provided with a chromatographic high pressure pump. Simultaneously 6% hydrogen peroxide solution is added to the reactor by the high pressure pump at the rate of 0.6 ml/min. Activity of the effluent solution and the leaching coefficients of strontium radionuclides from the layer of hydroxylapatite with synthesized calcium phosphate polycrystals which immobilized the radionuclides (charge), as specified upon completion of a test are given in Table 1

**Table 1**

| Solution, volume, ml | Strontium-90, activity, Ci/l |
|---|---|
| 100 | 1·10⁻¹⁰ |
| 500 | 6,7·10⁻¹⁰ |
| 1000 | 1,9·10⁻⁹ |
| 2500 | 4,1·10⁻⁸ |
| Leaching coefficient for charge, g/cm²·day | 1·10⁻⁵ |

EXAMPLE 2 (Variant 2). The bottoms of a nuclear waste evaporators which are purified from cesium radionuclides by filtration through ferrocyanide sorbents and contained cobalt-60 radionuclides (1·10⁻⁵ Ci/l) and manganese-54 (1·10⁻⁸ Ci/l) are passed through a layer of iron-cobalt ferrite (iron-cobalt oxides) with an iron to cobalt molar ratio of 1:01 and a particle size of 0.2-0.5 mm charged into a heated cylindrical reactor dimensioned 100 x10 mm. The process is carried out at the flow speed of 2 ml/min., at the temperature of 220°C and pressure of 100 atm (10.13 MPa). A solution flow is provided with a high pressure chromatographic pump. Simultaneously 6% solution of hydrogen peroxide is added to the reactor by the second high pressure pump at the rate of 0.6 ml/min. Activity of the effluent solution and the leaching coefficients of cobalt radionuclides from the charge of oxides formed, as specified upon completion of a test are given in Table 2.

**Table 2**

| Solution, volume, ml | Cobalt-60, activity, Ci/l | Manganese-54, activity, Ci/l |
|---|---|---|
| 100 | 1,4·10⁻⁹ | < 1·10⁻¹¹ |
| 500 | 1,1·10⁻⁹ | < 1·10⁻¹¹ |
| 1000 | 1,7·10⁻⁹ | < 1·10⁻¹¹ |
| 2500 | 1,5·10⁻⁹ | < 1·10⁻¹¹ |
| 5000 | 2,1·10⁻⁹ | < 1·10⁻¹¹ |
| Leaching coefficient for charge, g/cm²·day | 2·10⁻⁸ | < 1·10⁻⁷ |

EXAMPLE 3 (Variant 3). LRWs containing 2 g/l Trilon B and 0.5 g/l trisodium phosphate having a concentration of calcium ions of 0,1 g/l and comprising strontium-90 radionuclides (1.5·10⁻⁶ Ci/l) are passed through a layer of zirconium oxide having a particle size of 0.1-0.3 mm, charged into a heated cylindrical reactor dimensioned 100 x 10 mm. The process proceeds at the speed of a flow of 1 ml/min., at 200°C and the pressure of 10.13 MPa (100 atm). A solution flow is provided with a chromatographic high pressure pump. Simultaneously 6% solution of hydrogen peroxide is added to the reactor by a high pressure pump at the rate of 0.6 ml/min. Activity of an effluent solution and the leaching coefficients of strontium radionuclides from the charge of calcium phosphates and zirconium, as specified upon completion of a test are given in Table 3.

**Table 3**

| Solution, volume, ml | Activity, strontium-90, Ci/l |
|---|---|
| 100 | 1·1⁻¹⁰ |
| 500 | 1,8·10⁻⁹ |
| 1000 | 2,1·10⁻⁸ |
| Leaching coefficient for charge, g/cm²·day | 6·10⁻⁵ |

EXAMPLE 4. Sea water contaminated with strontium-90 radionuclides, 2·10⁻⁶ Ci activity, is passed through a layer of manganese dioxide having a particle size of 0.05-0.1 mm, charged in a heated cylindrical reactor dimensioned 100 x 10 mm. The process is carried out at the speed of a flow of 1 ml/min. at 220°C and the pressure of 10.13 MPa (100 atm). A solution flow is provided with a high pressure chromatographic pump. A solution 0.1 n manganese (II) chloride and 0.1 n potassium permanganate solution were added to the reactor by high pressure pumps at the rate of 0.6 ml/min. Activity of an effluent solution and the the leaching coefficients of strontium radionuclides from a charge of formable oxides as specified upon completion of a test are shown in Table 4

**Table 4**

| Solution, volume, ml | Activity, strontium-90, Ci/l |
|---|---|
| 100 | 5,6·10⁻⁹ |
| 500 | 4,0·10⁻⁹ |
| 1000 | 4,3·10⁻⁹ |
| 1500 | 4,5·10⁻⁹ |
| 2000 | 5,·10⁻⁹ |
| Leaching coefficient for charge, g/cm²·day | 1,4·10⁻⁷ |

EXAMPLE 5. LRWs being decontaminated containing 2 g/l sodium oxalate and 0.5 g/l Trilon B purified from cesium radionuclides by filtration through ferrocyanide sorbents and comprising cobalt - 60 (1·10⁻⁷ Ci/l) and strontium-90 (4·10⁻⁷ Ci/l) radionuclides are successively passed through a layer of iron-cobalt ferrite with a molar ratio of iron: cobalt of 1: 0.1 and a particle size of 0.2-0.5 mm, charged in a heated cylindrical reactor dimensioned 100 x 10 mm and through a layer of manganese dioxide having a particle size of 0.05-0.1 mm, charged in the heated cylindrical reactor dimensioned 100 x 10 mm. The process proceeds at the speed of a flow of 1 ml/min, at 200°C and pressure of 100 bar. A solution flow is provided a high pressure chromatographic pump. Simultaneously 6% hydrogen peroxide solution at the rate of 0.6 ml/min is added to the first reactor and 0.1 n manganese (II) chloride solution is added to the second reactor by the high-pressure pump. Activity of an effluent solution and

the leaching coefficients of cobalt radionuclides from formable oxides as specified upon completion of a test are shown in Table 5

**Table 5**

| Solution, volume, ml | Activity, cobalt-60, Ci/l | Activity, strontium-90, Ci/l |
|---|---|---|
| 100 | < 1·10-¹¹ | 1·10⁻¹⁰ |
| 500 | < 1·10⁻¹¹ | 1,4·10⁻¹⁰ |
| 1000 | < 1·10⁻¹¹ | 2,7·10⁻¹⁰ |
| 2500 | < 1·10⁻¹¹ | 1·10⁻¹⁰ |
| 5000 | < 1·10⁻¹¹ | 4.3·10⁻⁹ |
| Leaching coefficient for charge, g/cm²·day | 2·10⁻⁸ | 3·10⁻⁷ |

EXAMPLE 6. Alkali LRWs containing 0.3 g/l sodium hydroxide cobalt-60 (1·10⁻⁷ Ci/l) and cesium - 137 (6·10⁻⁷ Ci/l) radionuclides are passed through a layer of perlite-filter with the contained 3.4% iron, charged in a heated cylindrical reactor dimensioned 100 x 10 mm. The process is conducted at the speed of a flow of 0.3 ml/min. at 170°C and the pressure of 10.13 MPa (100 atm). A solution flow is provided with the high - pressure chromatographic pump. Activity of an effluent solution and the leaching coefficients of cobalt/cesium radionuclides from a charge of combined iron oxides and alumosilicates (faujasite in the main) as specified upon completion of a test are shown in Table 6.

**Table 6**

| Solution, volume, ml | Activity, cobalt-60, Ci/l | Activity, cesium-137, Ci/l |
|---|---|---|
| 100 | 7.4·10⁻¹⁰ | 2,1·10⁻⁹ |
| 200 | 2,1·10⁻¹⁰ | 7,8·10⁻¹⁰ |
| 500 | 4,2·10⁻¹⁰ | 1,1·10⁻⁹ |
| 800 | 7,9·10⁻¹⁰ | 1·10⁻⁹ |
| 1000 | 1,1·10⁻⁸ | 5,4·10⁻⁸ |
| Leaching coefficient for charge, g/cm²·day | 1·10⁻⁶ | 1·10⁻⁵ |
| Leaching coefficient for cement stone, g/cm²·day | 5·10⁻⁴ | 5·10⁻⁴ |

The afore-cited experimental data go to show that in treatment of LRWs by methods as claimed a charge representing either metal salts or metal oxides with immobilized storage suitable radionuclides is forming. A degree of leaching radionuclides is about 10⁻⁵·10⁻⁷ g/cm². day. The formed solutions are non-radioactive factory wastes.

## Claims

1. A method of reprocessing liquid radioactive waste LRW containing long-lived radionuclides by the synthesis of insoluble compounds immobilizing long-lived radionuclides into a crystal lattice, **characterized in that** the synthesis of a crystal phase is carried out under hydrothermal conditions at a temperature range from 180°C to 250°C and a pressure range from 2.026 to 15.2 MPa (20 to 150 atm) in a flow by passing LRWs being processed and reagents required for synthesis through a layer of iron oxide and/or manganese oxide and/or cobalt oxide and/or zirconium oxide at a rate providing for crystallizing of synthesizable radionuclide-containing compounds on the surface of the particles of the layer of oxides.

2. The method of reprocessing according to claim 1 **characterized in that** the crystal phase is synthesized as oxides and that the synthesizable radionuclide-containing compounds are oxides.

## Patentansprüche

1. Verfahren zur Aufbereitung von flüssigen radioaktiven Abfällen LRW, die langlebige Radionuklide enthalten durch die Synthese von unlöslichen Verbindungen, die die langlebigen Radionuklide in einem Kristallgitter immobilisieren, **dadurch gekennzeichnet, dass** die Synthese einer Kristallphase unter hydrothermalen Bedingungen in einem Temperaturbereich von 180°C bis 250°C und einem Druckbereich von 2,026 bis 15,2 MPa (20 bis 150 Atm) in einem Strom durchgeführt wird, indem die zu verarbeitenden LRW und die für die Synthese benötigten Reagenzien durch eine Schicht aus Eisenoxid und/oder Manganoxid und/oder Kobaltoxid und/oder Zirkoniumoxid mit einer Geschwindigkeit geleitet werden, die die Kristallisation von synthetisierbaren Radionuklid-haltigen Verbindungen auf der Partikeloberfläche der Oxidschicht gewährleistet.

2. Verfahren zur Aufbereitung gemäß Anspruch 1, **dadurch gekennzeichnet, dass** die Kristallphase als Oxide synthetisiert wird und dass die synthetisierbaren Radionuklid-haltigen Verbindungen Oxide sind.

## Revendications

1. Procédé de transformation de déchets radioactifs liquides DRL contenant des radionucléides à vie longue par la synthèse de composés insolubles immobilisant les radionucléides à vie longue dans un réseau cristallin, **caractérisé en ce que** la synthèse d'une phase cristalline est effectuée dans des conditions hydrothermiques, à une gamme de températures de 180 °C à 250 °C et une gamme de pressions de 2,026 à 15,2 MPa (20 à 150 atm.), dans un flux en faisant passer les DRL en cours de traitement et les réactifs requis pour la synthèse à travers une couche d'oxyde de fer et/ou d'oxyde de manganèse et/ou d'oxyde de cobalt et/ou d'oxyde de zirconium, à une vitesse permettant la cristallisation de composés synthétisables contenant les radionucléides sur la surface des particules de la couche d'oxydes.

2. Procédé de transformation selon la revendication 1, **caractérisé en ce que** la phase cristalline est synthétisée sous la forme d'oxydes et **en ce que** les composés synthétisables contenant les radionucléides sont des oxydes.
